

## UNITED STATES PATENT OFFICE

2,337,475

## PROCESS OF PREPARING ZINC AND CHLORINE

Ernst Kuss, Hans Hohn, and Fritz Stietzel, Duisburg, Germany; vested in the Alien Property Custodian

No Drawing. Application December 16, 1938, Serial No. 246,063. In Germany December 24, 1937

4 Claims. (CL 204—118)

This invention relates to the manufacture of zinc and chlorine by lixiviating chlorinated roasted zinc sulfide-containing materials.

Zinc and chlorine have already been obtained from the solutions resulting from the lixiviation of chlorinated roasted zinc sulfide-containing materials when subjecting the solutions after an intense purification to an electrolysis while using diaphragms. This process has not found any technical application for the following reasons:

The strongly electro-negative character of the zinc causes many troubles in the electrolysis, especially when impure solutions are used. Especially the electrolysis of zinc chloride solutions suffers from these troubles having an impairing effect on the yield. In this case especially iron and dissolved chlorine have a detrimental effect on the current yield. It has been tried to avoid these troubles by the use of diaphragms, the use of which, however, is connected with some disadvantages.

In accordance with the present invention we have found that it is unnecessary to proceed as mentioned above, i. e. to completely purify the solutions and to use diaphragms if carrying out the electrolysis with a mercury cathode. According to the invention zinc and chlorine are obtained from solutions, resulting from the lixiviation of chlorinated roasted zinc sulfide-containing materials while subjecting the solutions to the usual purification, by electrolyzing the zinc alkali metal chloride solution thus obtained while using a mercury cathode, by carrying away the chlorine evolved as gas and by separating the zinc from the amalgam produced.

As zinc sulfide-containing materials the cheap zinc-containing roasted pyrites can be used, which are obtained in large amounts in the manufacture of sulfuric acid. It is also possible to use zinc blends which are preferably mixed with roasted pyrites or other materials poor in zinc, the decomposition under these conditions being more complete and less subjected to troubles. This procedure also makes it possible to work up complex zinc ores, for instance complex lead-zinc ores, which generally are found connected with pyrites. The roasting process can be carried out in the usual manner. For the grade of purity of the solutions the required purity of the zinc obtained in the electrolysis is decisive, not the consideration of the current-yields, since slight impurities hardly diminish the current-yields in contradistinction to the working with solid cathodes. For instance, when electrolyzing a solution with about 20 mgrs. Fe, 20 mgrs. Co

and 10 mgrs. Ni to 100 grs. Zn, which could not possibly be worked up according to former methods, there is obtained by the use of a mercury cathode at a nearly theoretical current-yield a zinc having a purity of 99.98%. The purification, for instance, may take place in the following rather simple way: By cementation with iron copper and the noble metals are separated from the solutions, the sodium sulfate is separated by cooling, iron, cobalt, manganese, arsenic, antimony, etc., are precipitated by means of lime while oxidizing at the same time by means of chlorine at a pH beneath 6. As a result of this purification there are obtained zinc chloride solutions, containing alkali metal chloride as well as magnesium- and calcium-chloride. They are well suited for the electrolysis. The electrolysis by means of mercury cathodes can be carried out in the apparatus generally used in the industry. It is possible to work at room as well as at high temperatures. It is advisable to proceed in that way that the amalgam thus obtained remains liquid. The mercury is led in the same direction together with the solution through the cells. The zinc amalgam can be worked up electrolytically as well as thermally; it is advantageous to dissociate it by stages. The dissociation can take place in vacuo. The apparatus may work continuously or discontinuously. The mercury may be led in a closed circuit. Advantageously the amalgam is worked up continuously. While in the course of the known processes the exchange of the cathodes and the removing of the zinc plates do not allow an absolute continuous working, it is, on the other hand, possible to lead amalgam and the solution in a continuous stream through the cells when using mercury cathodes, without making it necessary to temporarily interrupt the working of the cells. In case the mercury is separated by distillation, this partial process in the same way as the process in question can be carried out continuously until the zinc is capable of being cast.

The invention is illustrated by the following examples:

## Example 1

Roasted pyrites of 57.10% Fe, 1.99% Cu, 2.39% Zn, 240 gms./ton Co, 300 gms./ton Mn, 0.04% Sb, 3.45% S, 0.11% As, 1.40% Pb, 4.05% SiO<sub>2</sub>, 62.0 gms./ton Ag, 1.02 gms./ton Au are after addition of 10% of sodium chloride, chlorinatingly roasted and lixiviated to produce a solution. This solution is decoppered by means of scrap iron and cooled to 0° C, to effect the removal of the bulk of

the sodium sulfate. The remainder of the sulfur together with Fe, As, Sb, Mn and Co are precipitated by means of lime while simultaneously introducing chlorine at a pH of 5.5. After filtration there is obtained a zinc chloride solution rich in sodium chloride, which contains magnesium- and calcium-chloride in small amounts. The zinc content amounts to 60 gms./liter. The solution is electrolyzed in cells, which are similar to the cells used in alkali metal chloride electrolysis, at a temperature of 70° C. and a current density of 1200 amp./m<sup>2</sup>. The electrolyte leaves the cells with a content of about 20 grams of zinc per liter. This zinc is precipitated with lime and the zinc hydroxide obtained is utilized in lieu of the calcium compound for the purification of the initial solution. The obtained chlorine gas is purified in the usual manner, dried and condensed. There is obtained an amalgam containing 4.5% of zinc, from which the mercury is distilled off. The zinc obtained is drawn off into casting molds; it has a purity of 99.95%.

*Example 2*

Roasted Meggen pyrites are mixed with copper containing roasted pyrites in a proportion of 1:1. The mixture contains 53.00% Fe, 0.55% Cu, 5.20% Zn, 240 gms./ton Co, 750 gms./ton Mn, 0.04% Sb, 0.14% As, 0.53% Pb, 8.30% SiO<sub>2</sub>, 3.95% S, 25.00 gms./ton Ag, 0.82 gms./ton Au. Sodium chloride in an amount of 12% is added to the mixture and according to the method of Example 1 a zinc solution containing 65 grams of zinc per liter is obtained. This solution is electrolyzed at a temperature of about 75° C. with a current density of 800 amperes per square meter while using amalgam cathodes. An amalgam containing 5% of zinc is produced in the electrolysis. Further treatment is effected in the manner described above.

We claim:

1. The process of preparing zinc and chlorine electrolytically which comprises subjecting a zinc sulfide-containing material to a chlorinating roast, lixiviating the roasted material, incom-

pletely purifying the resulting zinc chloride-containing solution to remove the sulfur and the main quantities of iron, cobalt, manganese, arsenic, antimony, nickel and other heavy metals which may be present so that the incompletely purified zinc chloride solution still contains alkali metal-, magnesium- and calcium-chlorides and iron, cobalt, and nickel to an extent whereby it is too impure to work up electrolytically with solid cathodes, and subjecting the said solution directly to electrolysis in a diaphragm-less cell with a liquid mercury cathode, recovering the chlorine as gas and separating the zinc from the mercury-zinc amalgam.

15 2. A process as in claim 1 in which the mercury as well as the solution are passed through the cell in the same direction.

20 3. A process as in claim 1 in which about 20 mgrs. iron, 20 mgrs. cobalt and 10' mgrs. nickel to 100 gms. zinc are present in the incompletely purified solution.

25 4. The process of preparing zinc and chlorine which comprises subjecting a zinc sulfide-containing ore to a chlorinating roast, lixiviating the roasted ore, decoppering the resultant solution by means of iron, cooling the solution to separate the bulk of sodium sulfate by crystallization, precipitating sulfur, iron, arsenic, antimony, manganese and cobalt by adding lime and simultaneously introducing chlorine at a pH of 5.5 and filtering, thereby obtaining an incompletely purified zinc chloride solution rich in sodium chloride, and which contains magnesium- and calcium-chlorides as well as iron, cobalt and nickel to an extent whereby it is too impure to work up electrolytically with solid cathodes, and subjecting the said solution to electrolysis in a diaphragm-less cell with a liquid mercury cathode, recovering the chlorine as gas and separating the zinc from the mercury-zinc amalgam.

ERNST KUSS.  
HANS HOHN.  
FRITZ STIETZEL.